

# UNITED STATES PATENT OFFICE.

FRANZ GATZSCHE, OF FREIBERG, GERMANY, ASSIGNOR TO THE "N. L." SYNDICATE, LIMITED, OF LONDON, ENGLAND.

## COMPOSITION FOR MAKING ARTIFICIAL LEATHER FABRIC.

SPECIFICATION forming part of Letters Patent No. 642,819, dated January 30, 1900.

Application filed October 8, 1898. Serial No. 893,036. (No specimens.)

To all whom it may concern:

Be it known that I, FRANZ GATZSCHE, a subject of the Emperor of Germany, and a resident of Freiberg; in the Kingdom of Saxony, Germany, have invented certain new and useful Improvements in Composition for Making Artificial Leather Fabric, of which the following is a specification.

The present invention has for its object a new composition for making artificial leather fabric, which fabric shall be cheaper than ordinary leather, but yet equally serviceable for use in the manufacture of various articles—such, for instance, as driving-belts.

15 The fabric consists in a strong felted material, preferably composed of hemp or of camel's hair, which is treated with my new composition, consisting of a mixture of glue, wax, oil, turpentine, and alcohol, as hereinabove specified.

In making the mixture the following proportions are preferred, though they may be varied somewhat, if desired: glue, one kilogram; wax, one kilogram; oil, one-half kilogram; turpentine, one-fourth kilogram; alcohol, one-half liter.

The glue is allowed to dissolve in thirty liters of water during one and a half days. The wax, oil, and turpentine are then added and 30 the mixture is boiled. Finally when the whole has cooled off under continuous stirring the alcohol is added and the mass is stirred to insure a perfect dissolution and thorough combination of all the ingredients.

The felt is immersed in this mixture, heated 35 to 80° centigrade, and is left until it is thoroughly impregnated therewith. It is then passed between rollers to press, stretch, and dry it and is finally varnished or lacquered. The product resembles ordinary leather and 40 is as strong as the latter and less liable to stretch.

The object of using the materials specified is as follows: The glue serves to produce an intimate combination of the separate molecules. The wax (preferably beeswax) serves to make the material, and consequently the belt, more pliable. The oil (preferably linseed-oil) serves to protect the material against the influence of the atmosphere, more especially against humidity, rain, &c. The turpentine serves to protect it against possible destruction by insects. The alcohol serves to dissolve the other ingredients.

Having thus described my invention, what 55 I claim, and desire to secure by Letters Patent, is—

A composition for making artificial leather fabric, consisting of a mixture of glue, one part; wax, one part; oil, one-half part; turpentine, one-fourth part, and alcohol, one-half part, as and for the purpose set forth.

Signed by me at Dresden, Saxony, this 19th day of September, 1898.

FRANZ GATZSCHE.

Witnesses:

ADOLF DAUM,  
HERNANDO DE SOTO.